

G. B. SHIPLEY.

METHOD OF IMPREGNATING TIMBER.  
APPLICATION FILED JUNE 27, 1914.

1,163,270.

Patented Dec. 7, 1915.



**WITNESSES**

W. T. Holman  
Glenn H. Leresche

**INVENTOR**

Grant B. Shipley,  
By Fredk H. Winter,  
Attorney.

# UNITED STATES PATENT OFFICE.

GRANT B. SHIPLEY, OF PITTSBURGH, PENNSYLVANIA.

## METHOD OF IMPREGNATING TIMBER.

1,163,270.

Specification of Letters Patent.

Patented Dec. 7, 1915.

Application filed June 27, 1914. Serial No. 847,730.

*To all whom it may concern:*

Be it known that I, GRANT B. SHIPLEY, a resident of Pittsburgh, in the county of Allegheny and State of Pennsylvania, have 5 invented a new and useful Improvement in Methods of Impregnating Timber, of which the following is a specification.

This invention relates to a method of preserving timber, and is more particularly 10 applicable to the treatment of railroad ties with a suitable preserving solution or composition.

The main object of the invention is to provide a method for treating ties and other 15 timber whereby a thorough penetration of the wood with a minimum amount of solution is secured, in order to reduce the weight of the ties or other timber, and whereby electric conductivity of the tie or timber, 20 the leaching or evaporation of the preserving solution, and corrosion of the spikes and tie plates is prevented, as well as other objects and advantages which will herein-after more fully appear.

25 Railroad ties have heretofore been treated with several preserving solutions, the principal ones being zinc chlorid and a coal tar product, universally called creosote in the trade. The creosote treatment is rather expensive, while the zinc chlorid treatment, 30 while less expensive is open to the objection that if the timber is thoroughly impregnated with the solution it is left very heavy, thereby not only increasing the difficulty of handling, but also the cost of transportation, and worse still, rendering the tie more or less electrically conductive, thereby destroying, or at least greatly reducing the efficiency of signaling systems now in use on 35 the railroads which make use of the track rails as conductors, which track rails must be insulated from each other by the ties. Furthermore, the zinc chlorid solution gradually evaporates and leeches out of the tie, 40 and also exerts a corrosive action on iron and steel, thereby causing undue corrosion of spikes, tie plates, etc.

The object of the present invention is to provide a method of treating timbers, and 45 particularly railroad ties, whereby the foregoing objections are overcome.

Generally stated, it consists in treating the ties or other timber, first with zinc

chlorid or other antiseptic salts, and afterward with a water-proofing composition 55 which may be the creosote above referred to or other coal tar product or a petroleum product, the treatment being so effected that the zinc chlorid does not produce the evil effects above noted, and the amount of preserving solution required is reduced to a 60 minimum.

The method may be carried out by various forms of apparatus, and the accompanying drawing shows merely diagrammatically 65 a single form or arrangement of apparatus by means of which the method may be carried out.

The apparatus may be of any design, but must comprise a suitable treating cylinder, 70 shown at 1, in which the timber is treated; an equalizing cylinder 2; two storage tanks, one tank 3 for containing the zinc chlorid or other preserving solution and the other tank 4 for containing the creosote or other 75 water-proofing composition; a pair of pressure and measuring tanks, one tank 5 for the preserving solution and the other tank 6 for the waterproofing composition, said tanks being mounted on scales indicated at 80 11, in order to secure accurate measurement of the solution or waterproofing compound absorbed by the timber; a compressor and vacuum pump 7; a condenser 8; a centrifugal pump 9; and an air pressure pump 85 10, together with suitable piping and valves connecting these parts arranged to circulate the solution and compound as required, and suitable coils in the retort and the several tanks for maintaining the necessary temperature for the best treatment of the timber, which coils will be connected up to a 90 boiler or other suitable means of steam pressure, not shown.

95 Preferably the equalizing cylinder 2 and waterproofing composition tank 4 are elevated above the treating cylinder 1 so that the preserving solution and waterproofing composition will flow by gravity into the treating cylinder. While in the drawing 100 only a single treating cylinder is shown as supplied from the equalizing cylinder, storage tanks and pressure tanks, it is obvious that any desired number of such cylinders can be connected by a suitable system of 105 piping.

As shown a pipe 12 leads from the bottoms of the tanks 2, 3 and 4, to the bottom of treating cylinder 1 and also to the pressure tanks 5 and 6, having a branch connecting to each of the latter. The air pressure pump 10 has its outlet 13 branched and connected to the tops of the pressure tanks 5 and 6. The centrifugal pump 9 has its inlet connected to the pipe 12 and its outlet connected by by-pass pipe 14 to the branch 12<sup>a</sup> running from pipe 12 to the equalizing tank 2. The pump 7 is arranged to act either as an air pressure or as a suction machine, being shown as a duplex compressor, having discharge pipes 15 connected through pipes 16 and 17 to the top of the treating cylinder 1 and being provided with a by-pass 18 in which is located the condenser 8 and by means of which said pump 20 is enabled to act as a suction or vacuum pump.

Suitable valves are located in various positions in the pipes of the system in order to effect the circulation of the preserving solution, the waterproofing composition and the air, as will hereinafter appear.

The treatment of the timber according to this process consists of two main steps or operations, viz., first treating the timber 20 with the preserving solution and afterward with the waterproofing compound. Before starting the system the cylinder 2 is filled with preserving solution from the storage tank 3, which is done by opening valves 19, 35 14<sup>a</sup> and 20 and closing valves 21 and 22, and starting the centrifugal pump 9. The pressure tank 5 is also filled with preserving solution from storage tank 3, and the pressure tank 6 is filled with water proofing compound from the storage tank 6. The cylinder 2 holds a little more preserving solution than is necessary to fill the treating cylinder 1.

The timber to be treated, indicated at 23, 45 is placed in the treating cylinder 1, and the latter is then sealed. The pump 7 is then started and valves 24, 25, 26 and 27 are opened and the valve 27<sup>a</sup> is closed, and the pump 7 acting as an air compressor forces 50 compressed air into the equalizing cylinder 2 above the preserving solution therein and also into the treating cylinder 1, where the air penetrates the pores or cells of the wood being treated.

55 When the pressure in the treating cylinder 1 and equalizing tank 2 reaches from 50 to 100 lbs. per sq. in. (depending upon the kind of timber being treated) the compressor 7 is stopped and the valves 20, 22, 28 and 29 are 60 opened whereupon the preserving solution flows by gravity from the cylinder 2 into the treating cylinder 1, displacing the air in treating cylinder 1 which passes through pipes 17 and 17<sup>a</sup> to the top of cylinder 2, without 65 reducing the air pressure and thus saving

pumping. Then the valves 20 and 28 are closed and the pressure on the top of cylinder 2 may be permitted to escape, such as through a bleed valve 30. The air pressure pump 10 is then started, the valves 13<sup>a</sup> 70 and 5<sup>a</sup> are opened and the valve 29 closed. The pump 10 compresses the air on top of the preserving solution in tank 5 and forces the solution into the treating cylinder 1 against a pressure which at the beginning is 75 from 50 to 100 lbs. per in., as above stated, and gradually increasing up to from 125 to 225 lbs. per inch, (depending upon the character of timber being treated) until no further solution can be forced into the timber. 80 The cylinder 1 is then drained, which is done by opening the necessary valves and by means of the air compressor pump 7 blowing the solution out of treating cylinder 1 and back into the cylinder 2. In the arrangement shown this is effected by closing valve 27<sup>a</sup>, opening valve 27 and closing valves 29, 25 and 21, and opening valves 26, 24, 28 and 29, whereby the solution is forced by the pump 7 back into the cylinder 2. 85

As soon as the treating cylinder 1 has been drained of the preserving solution the valves 28, 26, 25 and 27 are closed and the valves 24, 29, 31 and 27<sup>a</sup> are opened, and the pump 7 is again started, now acting as 95 a suction or vacuum pump to produce a quick vacuum in the treating cylinder 1 and withdraw from the timber from 30 to 50% of the fluid previously forced into the pores of the wood, which is collected in the 100 bottom of cylinder 1 and is returned through pipe 32 to the equalizing cylinder 2. The fluid withdrawn from the wood, by forming a partial vacuum in the treating cylinder, is somewhat weakened, and the solution remaining therein is correspondingly strengthened 105 by the processes of introducing and withdrawing the solution. In the preliminary step compressed air was forced into the pores of the wood, and was trapped in such 110 pores at the time the preserving solution was let into the treating cylinder 1 from the cylinder 2, and was further compressed when the preserving solution was forced into the pores of the wood by means of the 115 pressure pump 10. As soon as the pump 7 begins to act as a suction pump this trapped air expands and assists in forcing out of the wood the surplus water or weak solution, as a consequence of which the cells of 120 the wood instead of being left full of water or liquid solution merely have their walls coated with a thin film of the preserving solution. The operation thus leaves the timber thoroughly impregnated with a concentrated solution of zinc chlorid or other preserving salts to the amount of  $\frac{1}{2}$  to  $\frac{3}{4}$  lbs. per cubic foot of timber. The timber is 125 not therefore, in the heavy condition in which it is left by previous processes of 130

treating the same with zinc chlorid or similar preserving liquid, and furthermore since it contains a much smaller percentage of water is a better electrical insulator.

- 5 During the foregoing operations the treating cylinder and its contents are maintained at a temperature of from 140 to 180° Fahrenheit, by means of the steam coil 33 in the bottom of said retort, or if desired by 70 10 additional coils 34 in the cylinder 2 or coils 35 in the tank 3. The timber is then subjected to the second operation, viz., with the waterproofing composition from the tank 4. This is effected by closing the previously 75 15 open valves and opening valves 28, 29, 21 and 36, whereupon the waterproofing composition flows by gravity from tank 4 and fills the treating cylinder 1. All connections to the treating cylinder 1 are then closed 20 20 and valve 13<sup>b</sup> to the pressure tank 6 and valve 6<sup>a</sup> from pressure tank 6 are opened, and the air pressure pump 10 is again started. This creates pressure upon the waterproofing composition in tank 6 and forces additional 25 25 waterproofing composition from said tank into the treating cylinder 1 and into the timber contained therein. This pressure is continued until the timber has absorbed from 2 to 6 lbs. of the composition per cubic 30 30 foot, after which the pump 10 is stopped and the waterproofing composition is blown from the cylinder 1 and returned to the tank 4 by means of the compressor 7, in the same manner as heretofore described for returning the zinc chlorid solution to tank 2. 35 35 The valves are then again changed so as to convert the pump 7 into a suction or vacuum pump, and a vacuum is produced in the treating cylinder 1 in order to withdraw the surplus waterproofing composition from the timber, dry the latter, and prevent dripping, the surplus waterproofing composition being returned to the tank 6 through pipe 37. During the second treatment the waterproofing composition of coal tar or petroleum products is kept at a high temperature, substantially from 180 to 300° Fahrenheit, which can be effected by the heating coils 33 in the bottom of treating cylinder 1, or if 40 40 desired, by additional heating coils 38 in the tank 4 and 39 in the pressure tank 6. As a consequence, when the timber is removed from the treating cylinder and cools, the waterproofing composition on its exterior sets or hardens and therefore seals the cells of the timber and prevents the leaching out and evaporation of the preserving solution, with which the timber was treated in the first place, and also prevents the entrance of water and moisture into the timber and increases its chemical life. 45 50 55 60 65 70 75 80 85 90

By means of the foregoing method, timbers, and particularly railroad ties, can be expeditiously treated and in such manner that the entire body of the timber is im-

pregnated with a good preserving solution. At the same time the water of the solution is practically entirely withdrawn leaving the timber of relatively light weight, making it easier to handle and also reducing transportation charges. Furthermore, this treatment prevents the tie from becoming electrically conductive and therefore enables it to be used with automatic electric signaling systems. The waterproofing composition entirely coats the exterior and not only prevents loss of the preserving solution due to leeching and evaporation, but also when as usual the ties are gained and bored before treatment said waterproofing composition so coats the exterior of the tie and interior of the spike holes so that the plates and spikes are prevented from coming into contact with the zinc chlorid solution, which will prevent the corrosion of spikes and tie plates which occurs when the ties are treated with zinc chlorid, according to old processes. The process also gives a material saving in the cost of treatment as compared with the usual creosote treatment. 90

The process described is adapted for treating any character of wood or timber with a preserving solution and a waterproofing compound. While it has been described particularly for the treatment of railway ties, it is obvious that the process can be applied equally well to the treatment of paving blocks and various other forms of timbers which in use are subject to conditions which are likely to cause decay. 95

What I claim is:

1. The process of treating wood consisting in subjecting the wood to air pressure, and without relieving the air pressure subjecting the same to a bath of a preserving composition under a pressure higher than the air pressure, withdrawing the preserving composition and immediately subjecting the wood to a partial vacuum, thereby extracting a portion of water and composition, and then coating the wood with a waterproofing composition. 105
2. The process of treating wood consisting in subjecting the wood to air pressure, and without relieving the air pressure subjecting the same to a bath of a preserving composition under a pressure higher than the air pressure, withdrawing the composition, and immediately subjecting the wood to a partial vacuum, thereby extracting a portion of water and composition, and then subjecting the wood to a waterproofing composition under pressure. 110
3. The process of treating wood consisting in subjecting the wood to air pressure, and without relieving the air pressure subjecting the same to a bath of a preserving composition under a pressure higher than the air pressure, withdrawing the composition, and immediately subjecting the wood to a partial 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950

tial vacuum, thereby extracting a portion  
of water and composition, subjecting the  
wood to a waterproofing composition under  
pressure, and then withdrawing a portion of  
5 the waterproofing composition therefrom  
under a partial vacuum.

In testimony whereof, I have hereunto set  
my hand.

GRANT B. SHIPLEY.

Witnesses:

WILLIAM B. WHARTON,  
ELBERT L. HYDE.